

# UNITED STATES PATENT OFFICE.

WILLIAM W. SIMONSON, OF CINCINNATI, OHIO.

## ART OF REFINING KAOLIN AND SIMILAR CLAYS FOR USE IN MAKING POTTERY AND LIKE PRODUCTS.

1,185,254.

Specification of Letters Patent. Patented May 30, 1916.

No Drawing.

Application filed October 20, 1915. Serial No. 57,015.

*To all whom it may concern:*

Be it known that I, WILLIAM W. SIMONSON, a citizen of the United States of America, and a resident of Cincinnati, in the 5 county of Hamilton and State of Ohio, have invented a certain new and useful Improvement in the Art of Refining Kaolin and Similar Clays for Use in Making Pottery and like Products, of which the following 10 is a specification.

This invention relates to the process of decolorizing kaolin, bauxite, barite and allied materials that are used more particularly in the manufacture of white chinaware.

The principal object of the process herein is the removal of iron, such as oxid, or as hydrated oxid, from potters' clays in a simple, efficient, expeditious and economical 20 manner, and without any material detriment or injury to the clay itself or to the ware manufactured therefrom.

A very material object of the invention herein is the ready utilization of the hitherto wasted already-mined kaolin or clay that has been neglected and cast aside, adjacent the mine or bank deposits where it was but very poorly refined and with a loss of at 25 least 85% of the original raw material taken 30 from the mine or bank. It is well known to the art that immense quantities of said poorly or deficiently refined kaolin or clay are already lying broadcast and unused and awaiting just such a process as the one 35 herein to utilize or redeem them and to purge them of color and impurities and so that the actual residue-waste shall be practically *nil* or imperceptible. Thus, the labor required in actually mining the kaolin or 40 clay is materially lessened and saved, the unworked raw material or deposits in the mine or bank being really unnecessary to disturb for a long time to come and only 45 after said already-mined but defectively refined material is exhausted.

It is a well-known fact that the processes heretofore used and extant for removing iron-oxid from various clays involve the reduction of the ferric compounds to soluble 50 ferrous-salts and that the general or principal reducing agent has been sulfur-dioxid that becomes sulfuric-acid, or ferrous-sulfate combination simultaneously. Such reaction is exceedingly tardy and slow in 55 cases of primary clays used, and still slower

in cases of most of the secondary clays, and, in fact, is never really complete within the time-limits allowed for any successful and profitable industrial application.

The invention herein, therefore, contemplates the hastening or speeding of the reaction between iron-oxid and sulfurous-acid, which I have found in practice can be successfully accomplished by the employment of a small proportion of copper, the latter 60 being added as a soluble salt, either cupric or cuprous. In actual use by me, cupric-sulfate is employed, although, under certain conditions, the use of cupous-chlorid can be of greater advantage although not essential. 70 Now, however, whether beginning with a cupric salt or a cuprous salt, the end or termination of the solution of the iron-oxid finds most of the copper in solution as a cupric-salt, but always with a part present 75 as a cuprous-salt, a portion of which latter is in an insoluble state. Relatively small, this insoluble copper may be disregarded if the clay is to be used for facing paper or for other purely mechanical purposes, but 80 it may not remain in the clay if the same is to be used in the potter's mixtures. In order to remove this copper that is retained or held insoluble by the clay, an oxidizing 85 agent must be used and preferably in an acid bath, whereby this copper becomes dissolved as a cupric-salt and is afterward removed in a subsequent washing of the purified or refined clay with water.

The state of combination of the retained 90 copper is not known to a certainty, it amounting, however, to practically one part copper in five thousand of clay and as little as one part copper to twenty-five thousand of clay. It is known, too, that this copper 95 should not reach the pottery mixtures and that chlorin removes it from the clay, always as a cupric-salt (chlorid).

It will be observed that, at will, the products of the reaction, soluble after the iron 100 has been dissolved, may be readily washed away from the clay, and the insoluble cuprous salt then oxidized and washed away, while the cuprous salt itself may be oxidized in the presence of the soluble ferrous-salts, 105 and then the total metallic salts removed by a single washing. In either case, however, after the entire bulk of the soluble material has been washed away or removed by the use 110 of water, the partly washed clay is to be

given a wash of dilute acid and water, and this acid-wash then goes into the preparation of the next-acid-bath that is to be used on a later or succeeding quantity of clay.

5 This acid-bath is very material and useful in the process herein in order to fully avoid the retention by the clay of any part of the iron as a basic compound. Upon further washing with water, until the successive 10 washings shall give no response with testing re-agents for iron, the clay can be dried without disclosing or showing any stain or color on the surface of the dried cakes or masses thereof. It will be observed, at this 15 point, that the most convenient and best oxidizer for converting cuprous salts to cupric salts in this process is chlorin, which is preferably added as a gas to the aforesaid dilute acid-bath, in which latter the iron-free clay 20 is suspended.

The following formula for the iron-removing bath is one of the many possible ones that I claim as embodying my invention herein, the amount of copper employed being sufficient for practical and rapid work, a much less amount of copper not being practical nor useful, and a very material or greatly increased amount being really unnecessary:

|    |                    |      |        |             |
|----|--------------------|------|--------|-------------|
| 30 | Kaolin             | 2000 | pounds | avoirdupois |
|    | Sulfuric-acid, 77% |      |        |             |
|    | or 60 Baumé        | 40   | "      | "           |
|    | Sulfur-dioxid      | 12   | "      | "           |
| 35 | Cupric-sulfate     | 2    | "      | "           |
|    | Water              | 5000 | "      | "           |

The mass of clay is first mixed with the water until a smooth slip is obtained, the two acids being then added together with 40 the copper-salt, after all of them have been previously dissolved in water. The mixture is then heated to 60 degrees centigrade, or, if preferred, up to 90 centigrade, and then stirring until the iron-color has been sufficiently reduced or practically removed altogether. With the proportions thus given the operation will result in the removal of practically all the visible iron within a period of about four hours at the most. The 45 proportions of the said three re-agents of this formula can be varied to a considerable extent, those above-given applying to very badly or strongly colored clays and to a dissolving period of about four hours' time 50 that is to be considered as very rapid in the light of the many days' time heretofore required in producing even an inferior result, without the copper and bath, with the product still retaining a trace or hue of the iron-color therein, and which is not true of the 55 product resulting from my process herein.

The detail of washing the iron-free clay, and of acting upon it with chlorin, or with an equivalent of chlorin, may be considerably varied, as previously described.

I have further found that cuprous-chlorid alone will suffice to remove iron compounds from clays and like minerals when such are suspended in an acid-containing bath. To remove all of the iron it is necessary that 70 much more than the calculated amount of cuprous-chlorid be used than will be acted upon by the iron compounds as the air chiefly and other possible oxidizing agency or agencies will convert cuprous-chlorid to 75 cupric-chlorid under the working conditions. This alternative method is the more economical when copper as cuprous-chlorid can be recovered from low-grade copper ores by the well-known Hunt and Douglas 80 process, in which case the action of sulfur-dioxid precedes entirely the action of the cuprous-salt on the ferric compounds of the clays instead of going on concurrently with it. In the example of the iron-removing 85 bath previously given, 40 to 50 pounds of dry cuprous-chlorid would be used instead of the cupric-sulfate and sulfur-dioxid.

I claim:—

1. The process of removing iron from 90 clays, consisting in the employment of a solvent containing dilute acid and a cuprous salt.

2. The process of removing iron from 95 clays, consisting in the employment of a solvent containing dilute sulfuric-acid, sulfurous-acid and a salt of copper soluble in an acid solution.

3. In the process of removing iron from 100 clays, the use of salts of copper for hastening the reaction occurring between sulfurous-acid and iron compounds contained in said clays.

4. In the process of removing iron from clays, the combined action of an acid, a salt 105 of copper and a reducing agent able to convert ferric compounds to ferrous compounds.

5. The process of removing iron from 110 clays, consisting in the employment of a solvent containing dilute sulfuric-acid and cuprous-chlorid.

6. As an improvement in the art of refining kaolin for use in making pottery and like products, the herein-described process 115 of removing iron compounds from said kaolin consisting in the joint-action of an acid, a soluble salt of copper and a reducing-agent for converting ferric-oxid to ferrous oxid or salt.

7. The process of refining kaolin and similar clays for use in making white-ware and like pottery-products consisting in the employment of soluble copper salts for speeding or hastening the reaction that occurs between sulfurous-acid and ferric-oxid or hydrated, insoluble ferric compounds existing or occurring in said clays.

8. The process of removing iron from kaolin or like clay material in the puri-

ification or refinement thereof for its subsequent use in the manufacture of white-ware or like pottery-products consisting in the employment of a solvent that contains sulfuric-acid, sulfurous-acid and a copper salt soluble in an acid solution.

9. The process of removing iron from clays and like clay materials, consisting in acting upon the clay with a bath containing a mineral-acid, sulfurous-acid and a salt of copper, heated below the boiling-point of the bath until sufficient of the iron has been dissolved; then adding chlorin in excess of that taken up by the sulfur-dioxid and the cuprous and ferrous salts, and then washing the purified clay practically free from soluble compounds.

10. The process of removing iron from clays and like clay materials consisting in acting upon the clay with a bath containing a mineral-acid and a cuprous salt, heated below the boiling-point of the bath until sufficient of the iron has been dissolved, adding chlorin in excess of that taken up by the ferrous and cuprous salts, and then washing the purified clay practically free from soluble compounds.

11. The process of removing iron compounds from kaolin and other like clays for use in the manufacture of white pottery-products consisting in treating the clay with a bath containing sulfuric-acid, sulfurous-acid and a copper salt, such bath being heated below its boiling-point, then removing the dissolved iron salts and the accompanying re-agents, and then treating the

partially purified clay with a dilute acid, and with chlorin sufficient to be in excess of that used in the conversion of cuprous salt to cupric salt, and finally washing the refined clay so that it shall be practically free, from soluble compounds.

12. The process of removing iron from kaolin and other like clays used in the manufacture of chinaware or white pottery-products consisting in washing the clay in a bath of a mineral-acid, sulfurous-acid and a copper salt, the same being heated below its boiling-point until the iron has been dissolved therein, then adding chlorin in excess of that taken up by cuprous and ferrous salts, and then washing the purified clay until practically free from all soluble compounds.

13. The process of removing iron from clays and like clay materials, consisting in acting upon the clay with a bath containing dilute sulfuric-acid and cuprous chlorid, heated below the boiling-point of the bath, then removing the dissolved iron and copper and the accompanying re-agents of the bath and treating the partially purified clay with dilute-acid and chlorin in excess of that taken up by the cuprous compound retained by the clay, and then washing the refined clay practically free from soluble compounds.

WILLIAM W. SIMONSON.

Witnesses:

JOHN ELIAS JONES.

BERL B. RIGDON.